

## UNITED STATES PATENT OFFICE

HELLMUT FISCHER, OF BERLIN-FRIEDENAU, GERMANY, ASSIGNOR BY MESNE ASSIGNMENTS, TO METAL & THERMIT CORPORATION, OF NEW YORK, N. Y., A CORPORATION OF NEW JERSEY

## PROCESS FOR THE MANUFACTURE OF METALLIC BERYLLIUM OR ITS ALLOYS

No Drawing. Application filed October 3, 1927, Serial No. 223,835, and in Germany October 7, 1926.

This invention relates to a new process for the manufacture of metallic beryllium or its alloys by the electrolysis of molten materials, which process is suitable for the production 5 of beryllium or beryllium alloys both in a compact form and in the form of coatings.

Of the processes hitherto known for the manufacture of metallic beryllium the only one which has been found to be of any use 10 technically is that of Stock & Goldschmidt.

In this process the beryllium is separated by the electrolysis of molten materials from a molten mass composed of a mixture of double fluorides of beryllium with alkaline earth 15 metal fluorides and alkali metal fluorides.

The known process however is attended by difficulties inasmuch as on the one hand the preparation of the double fluorides required is a complicated and expensive procedure 20 and, on the other hand, a not inconsiderable loss frequently takes place during the working of the process owing to volatilization.

Similar difficulties are encountered in the manufacture of beryllium alloys or coatings 25 of beryllium when the above mentioned molten mass is employed.

The object of the present invention is to eliminate the aforesaid inconveniences. This is achieved according to this invention by 30 using as an integral part of the molten mass (instead of double fluorides) a simple oxygenated beryllium fluoride, that is, either basic beryllium fluoride or beryllium oxyfluoride mixed with one or more alkaline 35 earth metal fluorides with the addition if necessary of alkali metal halides.

By the term "basic beryllium fluoride" I designate such intermediate compounds, containing a greater or smaller proportion of 40 oxygen, which are formed during the preparation of beryllium oxyfluoride from normal beryllium fluoride,  $BeF_2$ . According to Lebeau (Comptes Rendus, vol. 126, 1898, page 1418) the formula for beryllium oxyfluoride is  $5BeF_2 \cdot BeO$ . So far as I am aware, no exact formulæ are available for basic beryllium fluoride.

The molten mass used in the new process, which contains a high percentage of beryllium, is considerably easier and cheaper to

prepare than the beryllium compounds used for the molten mass of the known process. The liability of the new molten mass to volatilizations is also considerably less. To supplement the electrolytically decomposed 55 beryllium salt, basic beryllium fluoride or beryllium oxyfluoride may be added as the process proceeds. The addition of alkali metal fluorides lowers the viscosity of the mass. If necessary beryllium oxide may also 60 be added to the new molten mass while the process is being worked. The solubility of the beryllium oxide in the new molten mass is considerably greater than it is in the molten mass employed in the older known process. 65 The oxygenated beryllium fluoride is preferably prepared separately and then mixed with the earth alkali metal fluoride.

The electrolysis of the molten substances is carried out according to the new process 70 conveniently at a temperature above the melting point of beryllium (i. e. about 1285° C.). The volatilization of the electrolyte is notwithstanding comparatively very slight at this temperature. A further and important 75 advantage of the new process is that the volatilizing salts, which in accordance with a further feature of the invention, are almost completely recovered, can be returned directly to the electrolysis again. The electrolysis of the molten substances when once made up and adequately saturated as the process proceeds with beryllium salts or flue dust can be carried on as long as may be desired. The new process therefore enables the 80 work to be carried on continuously, almost without any loss by volatilization, as, apart from slight losses in the volatilizing salts at the beginning only an addition of the beryllium salts decomposed by the electric current 85 is necessary.

To prepare compact metallic beryllium the new process may be carried out for example as follows:

A mixture of barium fluoride and beryllium 90 oxyfluoride is melted down in a suitable crucible, preferably of graphite, by the aid of the electric arc. The molten mass thus obtained and which may for example contain about 7% to 8% of beryllium, is brought to a temperature 100

above the melting point of beryllium, say about 1300° to 1350° C. for example and subjected to electrolysis at this temperature. In order to prevent the separated beryllium from being melted or burned, the cathode may be provided with means for cooling it by water. The beryllium is separated at the cathode in a very pure compact form. At suitable intervals of time as the bath becomes 10 poor in beryllium, beryllium oxyfluoride and if necessary some barium fluoride, the latter to replace the barium salt which has been volatilized, is added. The volatilized salts are trapped by means of a suitable apparatus 15 e. g. a dust chamber or on continuous current high tension electrodes, and the sublimation product either alone or if necessary together with fresh beryllium oxyfluoride used to make up the molten mass. The electrolysis can be 20 continued as long as may be desired only the beryllium regulus which is separated at the cathode must be removed from time to time according to the size of the bath in the crucible.

25 If the new process is to be used for the production of beryllium alloys, it is advisable to use the metal to be alloyed with the beryllium in the form of a liquid cathode and to otherwise carry out the process as in the 30 above example. To produce coatings of beryllium the article to be coated is introduced as a cathode into the molten mass and if necessary it may be cooled. In the production of beryllium coatings it is advantageous under 35 some circumstances, to use an intermediate layer which consists of another metal. Such intermediate layers may be produced galvanically for example and the metals and alloys which are best suited for this purpose 40 are those the melting points of which lie considerably above that of beryllium, e. g. tungsten, molybdenum, tantalum, vanadium, niobium, etc. Materials which are particularly suitable for the intermediate layer are iron, 45 copper, nickel, cobalt and others besides. After the intermediate layer has been applied to the article to be coated this latter is connected up as the cathode, introduced into the new molten mass and this latter then subjected to electrolysis at a temperature of 50 about 700° to 1200° C. It is also possible if it be required, to produce coatings of alloys of beryllium with or without an intermediate 55 layer. This may be done for example by adding the salt of a suitable alloying metal, such as aluminum for example, to the now molten mass. The metals which mainly are suitable for the production of beryllium alloys in a compact form or in the form of coatings 60 are aluminium, copper, magnesium, nickel, cobalt, iron etc.

What I claim as my invention and desire to be secured by Letters Patent is:—

1. In the production of electrodeposited 65 coatings containing beryllium, the process

which comprises electrolyzing a molten bath containing a beryllium compound selected from a class consisting of basic beryllium fluoride and beryllium oxyfluoride, and replenishing the bath by the addition of the 70 same said class of beryllium compounds, as such.

2. The process of claim 1 in which the said molten bath also contains compounds selected from a class consisting of alkaline earth metal 75 fluorides and alkali metal fluorides.

3. The process of claim 1 in which the beryllium compound employed is beryllium oxyfluoride.

In testimony whereof I affix my signature. 80  
HELLMUT FISCHER.

85

90

95

100

105

110

115

120

125

130